

# UNITED STATES PATENT OFFICE.

CHARLES BURROWS MOREY AND CHARLES JOSEPH HUBER, OF BUFFALO, NEW YORK,  
ASSIGNORS TO LARKIN CO., OF BUFFALO, NEW YORK.

## METHOD OF CLEANING METAL ARTICLES.

1,274,186.

Specification of Letters Patent. Patented July 30, 1918.

No Drawing.

Application filed June 23, 1917. Serial No. 176,601.

*To all whom it may concern:*

Be it known that we, CHARLES BURROWS MOREY and CHARLES JOSEPH HUBER, citizens of the United States, residing at Buffalo, in the county of Erie and State of New York, have invented a new and useful Improvement in Methods of Cleaning Metal Articles, of which the following is a specification.

This invention relates to methods of cleaning metal articles by immersing the same in an electrolyte in contact with a metal of more electro-positive properties than the metal to be cleaned.

In methods of this kind as heretofore employed it has been found that metal articles can only be successfully cleaned when the electro-positive metal is clean so that a good contact can be obtained between the articles to be cleaned and the electro-positive metal. The electro-positive metal, however, quickly becomes coated when immersed in electrolytes heretofore used so that in some cases it has been found necessary to employ a third metal for keeping clean the metal with which the article is to be cleaned is placed in contact.

The object of this invention is to provide an improved process of this kind in which the electrolyte itself keeps the electro-positive metal clean.

In carrying out this process any metal may be employed which is electro-positive with regard to the articles to be cleaned, zinc being preferably employed when silver or gold articles are to be cleaned. The electro-positive metal may be of any suitable form, a disk or plate being preferably employed which may be immersed in the electrolyte which should be contained in any suitable vessel or receptacle, preferably made of non-conducting material.

The electrolyte used in this process preferably consists of water in which is dissolved a sufficient quantity of some suitable salt to render the water a good conductor of electricity, about 3 per cent. of common salt or sodium chlorid having been found very satisfactory. Other salts may, however, be used if desired. A small amount of acid is then added to the electrolyte, approximately one-tenth of one per cent. (0.1%) having been found to produce satisfactory results. This acid may be of any suitable kind such as sulfuric, hydrochloric, acetic, or other acid which will not attack the articles to be

cleaned. This acid has the property of keeping the electro-positive metal clean by preventing the formation of a crust of salt or other deposit on the electro-positive metal. An electrolyte producing very satisfactory results can be made by dissolving one-half cup of salt in one gallon of hot water and adding thereto one-third cup of vinegar. The water should be as hot as the hands can readily bear.

The electrolyte thus formed is placed into a receptacle and the electro-positive body is placed on the bottom of the receptacle. The articles to be cleaned are then placed into the receptacle in contact with the electro-positive body, whereupon almost instantly after making contact they become clean. When the tarnish has been removed from the articles, they are removed from the electrolyte, rinsed, and if desired, polished with a chamois or flannel cloth.

The action which usually occurs in electrochemical processes of this kind appears to us that, when placed in the electrolyte, a difference of potential exists between the more electro-positive metal and the metal to be cleaned. When the metal to be cleaned and the more electro-positive one are brought into electrical contact, a circuit is established and an electrical current flows through the electrolyte from the more electro-positive metal to the metal to be cleaned, and with the flow of the electrical current nascent hydrogen forms on the surface of the metal to be cleaned. This highly active substance reconverts the tarnish and other metallic compounds to the simple metallic substance from which they were formed. It is therefore absolutely necessary that a good electrical contact be formed between the articles to be cleaned and the more electro-positive metal, otherwise no current will flow and no nascent hydrogen be produced.

By means of the method described the zinc or other electro-positive metal is kept clean by the action of the acid in the electrolyte and good electrical contact can be easily obtained, so that a large number of articles can be cleaned without producing any perceptible slowing down of the process or increase in the time required for cleaning the articles. The method is much simpler than those requiring the use of two metals in addition to the metal to be cleaned and produces thoroughly satisfactory results,

65

70

75

80

85

90

95

105

110

In the use of most methods employing an alkaline electrolyte with a zinc electro-positive electrode, a troublesome flocculent precipitate forms in the electrolyte which makes the solution more or less opaque. This difficulty is entirely removed by our acid method in which the solution remains clear and the process of cleaning can be readily observed.

10 While common salt or sodium chlorid has been found to be very satisfactory in this process, yet it is not intended to limit the invention to the use of sodium chlorid in the electrolyte, since any other salt having the property of rendering the liquid a conductor of electricity may be used, if desired.

15 We claim as our invention:

1. The herein described method of cleaning metal articles consisting in immersing the articles in an electrolyte containing an acid and in bringing the articles in contact while in said electrolyte with a metal of greater electro-positive character than the articles to be cleaned.

2. The herein described method of cleaning metal articles consisting in immersing the articles in an electrolyte consisting of water, a salt and an acid, in bringing the articles in contact while in said electrolyte with a metal of greater electro-positive character than the articles to be cleaned.

3. The herein described method of cleaning metal articles consisting in immersing the articles in an electrolyte consisting of water containing approximately three per cent. of salt and one tenth of one per cent. acid, and in bringing the articles in contact while in said electrolyte with a metal of greater electro-positive character than the articles to be cleaned.

4. The herein described method of cleaning metal articles consisting in immersing the articles in an electrolyte containing an acid and bringing the articles while immersed into contact with a body of zinc.

5. The herein described method of cleaning articles of silver, gold or the like, consisting in immersing the articles in an electrolyte consisting of water containing salt and vinegar in approximately the proportion of one-half cup of salt and one-third cup of vinegar to a gallon of water, immersing the articles in the electrolyte and bringing the same while immersed into contact with a body of zinc.

6. The herein described method of cleaning articles of silver, gold or the like, consisting in immersing the articles in a water solution containing approximately three per cent. sodium chlorid and one-tenth of one per cent. acetic acid, in bringing the articles while in said solution into contact with a piece of zinc also immersed in the solution, in removing the articles from the solution, in rinsing them and in polishing them.

7. The herein described method of cleaning metal articles consisting in immersing the articles in a hot solution consisting of salt and vinegar dissolved in water, and in bringing the articles while in said solution into contact with a metal of greater electro-positive character than the articles to be cleaned.

Witness our hands this 21st day of June, 1917.

CHARLES BURROWS MOREY.  
CHARLES JOSEPH HUBER.

Witnesses:

WILBUR L. KIRBY,  
HAL E. PUFF.